



US005601695A

**United States Patent** [19]**Muranushi**[11] **Patent Number:** **5,601,695**[45] **Date of Patent:** **Feb. 11, 1997**[54] **ETCHANT FOR ALUMINUM ALLOYS**[75] Inventor: **Yoshihisa Muranushi**, Yokohama, Japan[73] Assignee: **Atotech U.S.A., Inc.**, Somerset, N.J.[21] Appl. No.: **487,438**[22] Filed: **Jun. 7, 1995**[51] **Int. Cl.<sup>6</sup>** ..... **C25D 5/44**; C25D 3/12[52] **U.S. Cl.** ..... **205/213**; 205/252; 205/271[58] **Field of Search** ..... 205/214, 225, 205/252, 205, 139, 153, 185, 213, 271, 300, 183[56] **References Cited**

## U.S. PATENT DOCUMENTS

|           |         |                 |         |
|-----------|---------|-----------------|---------|
| 1,144,000 | 6/1915  | Roux            | 205/213 |
| 1,423,686 | 7/1922  | Schulte         | 205/300 |
| 2,162,789 | 4/1935  | Raub            | 205/213 |
| 2,436,690 | 3/1945  | Du Rose         | 205/271 |
| 2,511,952 | 6/1950  | Stareck et al.  |         |
| 2,580,773 | 1/1952  | Heiman          | 205/213 |
| 2,650,886 | 9/1953  | Zelley          |         |
| 2,709,847 | 6/1955  | Ihrie et al.    |         |
| 2,739,932 | 3/1956  | Forestek        |         |
| 2,746,136 | 5/1956  | Richaud         | 205/213 |
| 3,274,021 | 9/1966  | Jongkind et al. |         |
| 3,284,323 | 11/1966 | Leloup          |         |
| 3,321,328 | 5/1967  | Koretzky        |         |
| 3,505,179 | 4/1970  | Mander          | 205/213 |
| 3,594,197 | 7/1971  | Bunevich et al. |         |

|           |         |                   |         |
|-----------|---------|-------------------|---------|
| 3,622,470 | 11/1971 | Gowman            | .       |
| 3,881,999 | 5/1975  | Toth et al.       | .       |
| 4,018,949 | 4/1977  | Donakowski et al. | .       |
| 4,097,342 | 6/1978  | Cooke et al.      | .       |
| 4,100,038 | 7/1978  | Jongkind          | .       |
| 4,169,770 | 10/1979 | Cooke et al.      | .       |
| 4,192,722 | 3/1980  | Schardein et al.  | .       |
| 4,360,411 | 11/1982 | Ladet et al.      | 205/271 |
| 4,699,695 | 10/1987 | Rieger            | 205/213 |
| 5,246,565 | 9/1993  | Mignardot         | .       |

## FOREIGN PATENT DOCUMENTS

|         |        |                    |   |
|---------|--------|--------------------|---|
| 0278752 | 8/1988 | European Pat. Off. | . |
| 4429127 | 8/1995 | Germany            | . |

*Primary Examiner*—John Niebling*Assistant Examiner*—Alex Noguerola*Attorney, Agent, or Firm*—Finnegan, Henderson, Farabow, Garrett and Dunner, L.L.P.[57] **ABSTRACT**

A tin immersion composition of matter is disclosed comprising a compound comprising divalent tin ion, a compound comprising fluoride ion, and a compound comprising acid hydrogen ion. A process for treating an aluminum-copper or an aluminum-silicon alloy to improve the adhesion of metal layers to the alloy is also disclosed comprising contacting the alloy with an acidic tin immersion composition to produce a tin immersion coating on the alloy, and contacting the tin immersion coating with an etchant to substantially remove the tin immersion coating and produce an etched alloy surface.

**21 Claims, No Drawings**

## ETCHANT FOR ALUMINUM ALLOYS

## BACKGROUND OF THE INVENTION

## 1. Field of the Invention

The field of the invention is a composition of matter and a process for metal plating an aluminum surface.

## 2. Description of Related Art

Harrison et al. in an entitled article "Plated Aluminum Wheel Characterization," *Metal Finishing*, December 1994, pp. 11-16, notes that metal plating aluminum is one of the growing areas of decorative plating, especially aluminum automobile wheels. Although in the past plated aluminum wheels were a small after-market specialty item, this has become an original equipment manufacturer option and a special addition feature.

The major concerns in production of metal plated aluminum are the reliability of the plating process, appearance and cost.

In a typical sequence for applying metal coatings to aluminum, the substrate is polished and soak cleaned. The soak cleaner employed in the pretreatment of the aluminum surface removes finishing oils, grease and difficult-to-remove buffering compounds left on the surface of the aluminum from polishing.

After the soak clean, the aluminum is immersed in a mild caustic or alkaline etch solution operated at elevated temperatures since etch rate is more dependent on temperature than caustic concentration.

The mild alkaline etch removes the Beilby layer and roughens the surface. Employing aluminum-silicon alloys results in etching aluminum preferentially over the silicon, leaving coarse silicon crystals exposed on the surface.

An examination of the surface of the aluminum-silicon alloy shows large areas of exposed silicon interspersed within the aluminum matrix. The silicon particles vary in size, do not appear to be uniformly distributed throughout the casting, and are not uniformly distributed on the surface of the aluminum, but rather in discrete areas. Silicon crystals protrude from the surface, most of which are oriented perpendicular to the surface.

After the etch treatment, the substrate is then subjected to a desmut composition. Smaller, loosely adherent silicon particles (where a silicon containing alloy is employed), as well as intermetallic compounds, are most likely removed during the desmut step. The substrate is then rinsed, zinced, stripped with nitric acid, zinced again, and followed by a nickel strike coating. This in turn is followed by a bright copper plating, optional copper buffering, nickel plating and an optional high sulfur nickel to improve corrosion resistance. After these preparatory steps, a decorative chromium plate is applied.

As noted by Harrison et al., a film is left on the aluminum after the mild caustic etch that is removed by the desmut step, and is one of the most crucial steps in processing the aluminum substrate to ensure adequate adhesion of the subsequently applied metal coatings. The tenacity of this film varies with the composition of the aluminum, especially where an aluminum alloy is employed.

The desmut solution contains strong mineral acids, and when aluminum-silicon alloys are treated, fluoride ions. Both are selected to uniformly attack the aluminum surface, or the proportions varied to preferentially dissolve the silicon (e.g., high fluoride concentration) and/or the aluminum. The aluminum and exposed silicon particles are

thereby rendered more active. Various combinations of additives, nitric, sulfuric, and phosphoric acids in combination with fluoride salts such as ammonium bifluoride or fluoroboric acid allow for adequate pretreatment of the aluminum to obtain good adhesion of subsequently applied metal coatings.

Aluminum wheels employed by the automotive industry are generally A-356 aluminum alloy castings. The A-356 alloy is generally chosen for aluminum wheel applications because of its ease of use in casting, high resistance to hot cracking, high fluidity, low shrinkage tendency and moderate ease of machinability.

The A-356 alloy is a hypoeutectic alloy consisting mainly of a two-phase microstructure. Iron is present to minimize sticking between the molds and casting. Magnesium and copper are added to impart strength to the alloy. Manganese is believed to improve the high temperature properties of the casting. The silicon in the alloy appears as very hard particles and imparts wear resistance. Most of the hypoeutectic aluminum-silicon alloy consists of a soft and ductile aluminum phase.

The nominal composition of A-356 aluminum alloys is as follows:

|    | Element | % by weight |
|----|---------|-------------|
|    | Al      | 91.9        |
|    | Si      | 7.0         |
|    | Cu      | 0.2         |
|    | Mg      | 0.3         |
| 30 | Mn      | 0.1         |
|    | Zn      | 0.1         |
|    | Fe      | 0.2         |
|    | Ti      | 0.2         |

Treating aluminum alloys such as A-356 alloy in the foregoing manner leaves a heavy film on the aluminum after the mild caustic etch. This film or smut is a mixture of both aluminum oxides and alloying element oxides as well as exposed silicon in those alloys which contain silicon as an element.

The zinced materials generally consisted of CN zinc compositions that optionally contained nickel, and because of environmental reasons and the state-of-the-art cyanide treatment technology, manufacturers sought cyanide free systems.

Several cyanide free zinced compositions have been developed containing zinc and optionally nickel, copper, or iron and mixtures thereof; however, it was found in some instances that specific aluminum alloys, such as A-356 alloy, could not be pretreated satisfactorily in that a heterogeneous composition was formed on the surface of this alloy during the initial etch, sometimes referred to as segregation. This segregation in turn has an adverse affect on the adhesion of subsequently applied metal layers.

It was further found that aluminum-copper alloys such as 2024 alloy could not be etched uniformly either by alkaline or acid etchants due to its low solution potential. It was also found that this compromised the adhesion of subsequently applied metal coatings.

Ullman's Encyclopedia of Industrial Chemistry, Vol. A-1, p. 520 (1985), notes that the nature of the aluminum oxide surface and reactivity of aluminum after oxide removal makes electroplating more complicated. Additional factors include reactions between aluminum and the electroplating solutions, the galvanic reactions between aluminum and the plated metal, and the metallurgical structure of aluminum

alloys that consists of solid solutions, constituents, disper-  
soids, and precipitates, each having a different reactivity.

As is apparent from the foregoing, metal plating of  
aluminum surfaces is a highly complex field.

It would therefore be an advantage to provide a process or  
composition for avoiding or minimizing the difficulties of  
smut formation, segregation, nonuniform etching and poor  
adhesion in the electrocoating of aluminum substrates in a  
process that utilizes cyanide-free zinc compositions.

Accordingly, the present invention is directed to a com-  
position of matter and a process that substantially obviates  
one or more of these and other problems due to limitations  
and disadvantages of the related art.

#### SUMMARY OF THE INVENTION

These and other advantages are obtained according to the  
present invention.

Additional features and advantages of the invention are  
set forth in the description that follows, and in part are  
apparent from the description, or learned by practice of the  
invention. The objectives and other advantages of the inven-  
tion are realized and obtained by the composition of matter  
and process particularly pointed out in the written descrip-  
tion and claims hereof.

To achieve these and other advantages, and in accordance  
with the purpose of the invention, as embodied and broadly  
described herein, the invention comprises a novel acidic tin  
immersion composition of matter comprising a divalent tin  
ion-containing compound, a fluoride ion-containing com-  
pound, and an acid hydrogen ion-containing compound.

The invention also comprises a process for treating an  
aluminum-copper or an aluminum-silicon alloy to improve  
the adhesion of metal layers to the alloy comprising:

- (a) contacting the alloy with an acidic tin immersion  
composition to produce a tin immersion coating on the  
alloy;
- (b) contacting the tin immersion coating with an etchant  
to substantially remove the tin immersion coating to  
produce an etched alloy surface.

The substrate, and especially an aluminum-copper sub-  
strate is simultaneously etched and coated with the acidic tin  
immersion coating, and especially the novel acidic tin  
immersion coating of the invention. This is preferably  
followed by a separate etching step to substantially remove  
the tin immersion coating and provide a microporous struc-  
ture on the surface of the aluminum alloy.

In another embodiment, an aluminum silicon containing  
substrate is coated with the acidic tin immersion coating,  
especially the novel acidic tin immersion coating of the  
invention, again to simultaneously etch and deposit a tin  
immersion coating on the aluminum alloy. A fluoride etchant  
applied to the tin coating on the aluminum substrate sub-  
stantially removes the tin immersion coating and produces a  
microporous structure on the aluminum surface.

A cyanide-free zinc immersion coating is then applied to  
the aluminum substrate followed by electrodeposition of a  
metal layer such as nickel. The microporous structure pro-  
duced by the acidic tin immersion coating/etching process  
provides improved adhesion for subsequently applied metal  
layers.

#### DETAILED DESCRIPTION OF THE INVENTION

The invention comprises a novel acidic tin immersion  
coating composition having a fluoride ion-containing com-

ound, and is employed in a process that provides a  
microporous structure on an aluminum substrate.

Employing an acidic tin immersion coating, and espe-  
cially the novel acidic tin immersion composition of the  
invention having a fluoride ion-containing compound allows  
for the subsequent uniform etching of the aluminum sub-  
strate to substantially remove the tin to obtain an etched  
aluminum substrate, and especially a microporous structure  
on the substrate that promotes improved adhesion of sub-  
sequently applied metal coatings. The process of the invention  
is especially applicable to aluminum-copper alloys and  
aluminum-silicon alloys. Where the latter is employed,  
etching the tin immersion coating is preferably carried out  
using a fluoride ion containing etchant.

After substantial removal of the tin immersion coating  
from the aluminum surface by etching, the aluminum sur-  
face may be coated with a metal by an immersion or  
electrolytic process. Alternatively the etched or metal coated  
aluminum substrate may be coated with a metal using other  
methods known in the art, such as non-immersion methods  
and non-electrolytic methods, including cathode sputtering,  
chemical vapor deposition (CVD), ion beam coating and the  
like. Any metal may be coated in this regard such as zinc,  
chromium, copper, nickel, or combinations thereof, whether  
alloy combinations, or multiple layers of the same or dif-  
ferent metals or alloys.

The preferred process of the invention comprises coating  
an aluminum-copper or aluminum-silicon alloy substrate  
with the novel acidic tin immersion composition having a  
fluoride ion-containing compound. This is followed by sub-  
stantially removing the tin coating on the aluminum by  
etching, and optionally coating with a metal. An etchant  
having a fluoride ion-containing compound is preferred for  
etching the aluminum-silicon alloy coated with the tin  
immersion coating.

The novel acidic tin immersion coating of the invention  
and process is especially effective for plating an aluminum-  
copper alloy or an aluminum-silicon alloy substrate in a  
process that utilizes a cyanide free immersion zincating step  
or steps, followed by the electrolytic application of a metal  
layer or layers, such as zinc, chromium, copper, nickel, or  
combinations thereof, whether alloy combinations, or mul-  
tiple layers of the same or different metals or alloys.

Throughout the specification, reference is made to alum-  
inum-copper alloys by which it is intended to include any  
alloys of aluminum and copper where copper is present in an  
amount greater than about 1% by weight. Similarly, refer-  
ence herein to aluminum-silicon alloys is intended to include  
those alloys of aluminum and silicon in which the silicon is  
present in an amount greater than about 1% by weight.

The process of the invention is broad enough to include  
the application of any acidic tin immersion coatings to the  
aluminum surface and especially the surface of the alum-  
inum-copper alloys and the aluminum-silicon alloys as  
defined herein. The acidic tin immersion coatings are further  
described by Shipley, U.S. Pat. No. 3,303,029; Ceresa et al,  
U.S. Pat. No. 2,891,871; Sullivan et al, U.S. Pat. No.  
2,369,620; and Bradley, U.S. Pat. No. 2,282,511, all of  
which are incorporated herein by reference. The present  
invention includes a process employing these types of tin  
immersion coatings applied to an aluminum substrate,  
etched to substantially remove the tin immersion coating,  
and especially where the etched aluminum is coated with a  
metal layer by any of the processes described herein.

In the preferred embodiment of the invention, the alum-  
inum surface produced by acidic tin immersion coating

followed by etching to substantially remove the tin immersion coating comprises a microporous surface. Such a microporous surface is produced by this process, and especially the process employing the novel acidic tin immersion coating of the invention.

Prior to the present invention, it was found that aluminum-copper alloys such as alloy 2024 were not etched uniformly either by alkaline or acidic etching materials because of its low solution potential. Employing the novel acidic tin immersion coating of the invention in lieu of a first cyanide free zincating step, followed by etching to substantially remove the tin immersion coating, provides a microporous structure, and uniform etching of the surface of alloy 2024.

The process comprised soak cleaning alloy 2024 in a commercially available cleaner (Atotech Alkleen™-All), etching in an alkaline etch (Alkleen™ A-77), followed by a commercial nitric acid desmut material. A commercially available cyanide free zincate coating was then applied (Tribon™, M&T Harshaw Japan), followed by nitric acid stripping, Tribon™ zincating and Watts nickel plating. By employing the novel acidic tin immersion coating of the invention in lieu of the first Tribon™ zincating step in this process, uniform etching was achieved and the adhesion performance improved.

Alloy A-380 (Al—Si—Cu alloy) was treated satisfactorily by this process as well.

It was also discovered that alloy A-356 was not pretreated satisfactorily with the existing cyanide free zincate process. The use of the a fluoride containing etchant on the aluminum substrate to replace Alkleen™ A-77 alkaline etchant and the nitric acid desmut composition still did not improve adhesion sufficiently. It appears that this is caused by the formation of a heterogeneous composition on the surface of the A-356 alloy, referred to as segregation.

It was discovered that by applying the novel acidic tin immersion coating of the invention to the A-356 alloy, simultaneously etches it and produces a tin immersion coating on the surface. The tin immersion coating is then substantially removed by applying a fluoride etchant to the surface, resulting in uniform and deep etching to reduce the effect of segregation. A thin passivated film also forms on the surface that inhibits rapid zinc deposition in the zincating process.

In coating the A-356 alloy, a sequence of steps is employed comprising soak cleaning the aluminum substrate in Alkleen™ A-11, followed by applying the acidic tin immersion coating to provide a microporous surface on the aluminum substrate. The surface thus obtained is then treated with a special etchant followed by Tribon™ zincating, nitric acid stripping, Tribon™ zincating, and Watts nickel plating.

This process provides superior adhesion of the metal layers subsequently applied to the A-356 alloy by electrolytic means, such as Watts nickel.

Besides improving adhesion, the novel acid tin immersion coating of the invention has another advantage of lowering the cost of the treatment, and is also easily treated in any waste water because it contains no chelating agent and is cyanide free.

The acidic tin immersion coating is preferred for coating aluminum-copper alloys and aluminum-silicon alloys for several reasons. Zinc, which has an oxidation potential of -0.763 V, is satisfactorily applied to magnesium-rich aluminum alloy 5052 or pure aluminum 1100 that have an oxidation potential of -0.83 V but is not readily coated onto

a copper-rich aluminum alloy such as alloy 2024 that has an oxidation potential of -0.66 V. Divalent tin, however, has an oxidation potential of -0.136 V and is readily coated onto these aluminum copper alloys as well as aluminum silicon alloys.

Although nickel has an oxidation potential of -0.250 V and will readily enter into an immersion reaction with copper-rich aluminum, it is unacceptable because it produces a dense replacement layer and blocks further reaction.

Although the inventor does not wish to be limited by any theory, it is believed that the acidic tin immersion coating produces a spongy replacement layer that does not block further reaction of the tin coating. This, therefore, allows continuing replacement layer growth at uncovered locations on the aluminum substrate leading to microporosity. As noted, nickel, in contrast, produces a dense replacement layer and blocks further reaction.

The novel acidic tin immersion coating of the invention provides a highly porous surface on the aluminum, and it is believed this surface results from the immersion or substitution reaction between tin and aluminum. As noted before, other metal ions did not produce the same degree of microporosity in the substitution or immersion reaction.

The novel acidic tin immersion coating of the invention acts in some respects as an acid etching solution, as well as an immersion coating to provide a tin layer on the aluminum alloy substrates. In the process of the present invention, this tin coating is subsequently etched, and the tin stripped away in part or completely, described herein as the substantial removal of tin. The stripping step leaves an exposed aluminum alloy surface that has a unique microporous surface that is further coated with a metal as described herein, and especially with cyanide free zinc immersion coatings.

The application of the acidic tin immersion coating is undertaken, not to produce a lasting tin coating, but to create a microporous structure on the surface of the aluminum.

The acidic tin immersion tin composition having a fluoride ion-containing compound comprises a divalent tin salt such as tin sulfate or any other equivalent salt of tin. These salts are the reaction product of tin compounds with an acid such as a mineral acid including the acids based on oxides of sulfur, phosphorus or nitrogen as well as organic acids, or halogen acids such as acids based on fluorine, chlorine, bromine and iodine.

In addition to sulfuric acid, the mineral acids include sulfurous acid, nitric acid, nitrous acid, phosphoric acid, phosphonic acid, phosphinic acid and the halogen acids such as hydrochloric, hydrofluoric, hydrobromic and hydroiodic acids, all of which are known in the art.

The organic acids in this regard comprise any monocarboxylic or polycarboxylic acids such as the dicarboxylic, tricarboxylic or tetracarboxylic acids known in the art. Examples include the aliphatic acids, cycloaliphatic acids and aromatic acids where the aliphatic acids contain from 1 to about 5 carbon atoms and the cycloaliphatic and aromatic acids contain from 6 to about 10 carbon atoms, and include acids such as acetic, hydroxyacetic acid, maleic acid, malic acid, phthalic acid, mellitic acid, trimellitic acid, benzoic acid and the like. Mixtures of acids can be used, including the two, three, or four component mixtures.

The preferred acid comprises a mineral acid, and especially sulfuric acid. Preferred tin salts comprise tin sulfates.

The acidic tin immersion coating of the invention has a fluoride ion-containing compound where the source of the fluoride ion can be hydrogen fluoride or any fluoride salt

such as ammonium bifluoride, aluminum trifluoride, sodium fluoride, sodium bifluoride, potassium bifluoride, ammonium fluoride, fluoroboric acid or hydrofluoric acid. Ammonium bifluoride or ammonium fluoride are not ordinarily employed where ammonia fumes are a potential irritant. The alkali metal fluorides and hydrofluoric acid are especially suitable in this regard. Mixtures of the various compounds that will provide fluoride ion can be employed, especially the two, three, or four component mixtures.

The acid hydrogen ion-containing compound is based on an acid as described herein, and especially the mineral acids. Preferred acids are those having the same anion as the tin salt.

The ratios of divalent tin ion, fluoride ion and acid hydrogen ion of the novel acidic tin immersion composition are selected to provide both etching and a tin immersion coating on the surface of the aluminum that will produce the desired microporous structure of the invention. The divalent tin ion generally is present in an amount from about 0.05 to about 0.15 mols and especially from about 0.075 to about 0.125 mols. The compound containing the fluoride ion is employed in the immersion composition so that the fluoride ion is present in an amount from about 0.25 to about 0.75 mols and especially from about 0.375 to about 0.625 mols. Lastly, the acid is selected so that the acidic hydrogen ion in the composition is anywhere from about 0.25 to about 0.75 mols and especially from about 0.375 to about 0.625 mols.

These molar amounts of the ionic species are also the gram atoms of the ionic species employed, and take into account that some of the compounds that are used to provide these ionic species contain more than one gram atom of the particular ionic species per mol. For example, sulfuric acid contains two gram atoms of hydrogen per mol, whereas hydrochloric acid contains one gram atom of hydrogen per mol. Consequently, the quantities of the various components have not been expressed as molar amounts of the compounds employed, but rather the molar amounts of the ionic species contributed by the compounds.

Although the foregoing molar amounts are used to define the ratios of the various divalent tin ion, fluoride ion and acid hydrogen ion, they also indicate the concentration of an aqueous tin immersion composition in that these molar amounts comprise the quantity of the components of the immersion composition that can be employed in one liter of water to make up the immersion composition.

The etchant employed for removing the acidic tin immersion coating from the aluminum-silicon alloy comprises a composition having a fluoride ion-containing compound, the latter comprising any of the fluoride ion-containing compounds described herein. This etchant also includes these fluoride ion-containing compound used in combination with an acid such as a mineral acid as defined herein.

The following examples are illustrative.

A novel acidic tin immersion coating of the invention (also referred to as Microporous Etch) is prepared as follows:

|                                 |              |
|---------------------------------|--------------|
| $\text{SnSO}_4$                 | 21.5 g/liter |
| HF (47%)                        | 20 ml/liter  |
| $\text{H}_2\text{SO}_4$ (95.0%) | 5.2 ml/liter |

Two standard process sequences were used to plate various aluminum substrates as follows.

In these processes, the zincate was a standard cyanide-free zincate solution containing zinc ions and optionally nickel, copper and iron ions.

Cyanide free zinc immersion coatings for aluminum are described by Stareck, U.S. Pat. No. 2,511,952; and Ihrie et al, U.S. Pat. No. 2,709,847. Zelley, U.S. Pat. No. 2,650,886 describes a zinc-iron cyanide-free zinc immersion coating for aluminum. Any of the foregoing zinc immersion coatings can be employed and modified to include in addition to iron, nickel, copper or any combination of nickel, copper and iron with zinc in the zinc immersion coatings. This modification is easily made by a person of ordinary skill in the art.

Unless otherwise indicated, the desmut process was carried out with a composition comprising a mineral acid desmut composition as described herein comprising a fluoride ion-containing compound such as hydrogen fluoride or any fluoride salt as described herein. This desmut process, when applied to the acidic tin immersion coating, has also been referred to herein as an etching step.

The nickel plating comprised the application of a nickel coating by means of a Watts bath well-known in the art.

#### Example 1.

##### Process A

1. Soak Clean (Alkleen™ A-11)
2. Alkaline etch (Alkleen™ A-77)
3. Desmut (Cleaner #30; Acidic product  $\text{HNO}_3$  and  $\text{H}_2\text{SO}_4$  for silicon containing Al-alloy)
4. Zincate
5. Zincate-removal ( $\text{HNO}_3$ , 50% Vol)
6. Zincate
7. Ni Plating

##### Example 2.

##### Process B

1. Soak Clean (Alkleen™ A-11)
2. Desmut
3. Zincate
4. Zincate removal ( $\text{HNO}_3$ , 50% Vol)
5. Zincate
6. Nickel Plating

##### Adhesion Results:

|                    | Process A | Process B |
|--------------------|-----------|-----------|
| **Pure Aluminum    | 1100      | Good      |
| **Cu-Rich Aluminum | 2024      | Poor      |
| **Mg-Rich Aluminum | 5052      | Good      |
| *Al-Si Alloy       | A-356     | Poor      |
| *Al-Cu-Si-Alloy    | A-380     | Poor      |

\*Cast material

\*\*Extruded material

As can be seen from the foregoing, poor results were obtained for aluminum alloys containing copper or silicon.

Accordingly, processes A and B were modified to include the novel acidic tin immersion composition of the present invention containing fluoride. This composition is described as a Microporous Etch in the following examples:

#### Example 3

##### Process A Modified.

1. Soak Clean (Alkleen™ A-11)
2. Alkaline Etch (Alkleen™ A-77)
3. Desmut (Cleaner No. 30)
4. Microporous Etch
5.  $\text{HNO}_3$  (50% vol)
6. Zincating
7. Ni Plating

## Example 4

| Process B modified.   |                              |      |
|-----------------------|------------------------------|------|
| 1. Soak Clean         | (Alkleen™ A-11)              |      |
| 2. Microporous Etch   |                              |      |
| 3. Desmut             |                              |      |
| 4. Zincating          |                              |      |
| 5. Zincate-removal    | (HNO <sub>3</sub> , 50% vol) |      |
| 6. Zincating          |                              |      |
| 7. Ni Plating         |                              |      |
| Process A Modified    | Process B Modified           |      |
| Pure Aluminum 1100    | Poor                         |      |
| Cu-Rich Aluminum 2024 | Good                         |      |
| Mg-Rich Aluminum 5052 | Poor                         |      |
| Al-Si Alloy A-356     | Poor                         | Good |
| Al-Cu-Si Alloy A-380  | Good                         |      |

The desmut, zincating and nickel plating steps employed were the same as in Examples 1 and 2. As can be seen from the results employing modified processes A and B, good adhesion to copper and silicon containing aluminum alloys were obtained by employing the composition and processes of present invention.

Where tin deposition is too fast, thereby impairing the formation of an acceptable microporous structure, an organic compound, such as gelatin, can be added to the novel acidic tin immersion composition containing fluoride.

It will be apparent to those skilled in the art that modifications and variations can be made in the novel composition of matter and process for a coating in aluminum substrate of the present invention without departing from the spirit or scope of the invention. It is intended that these modifications and variations and their equivalents are to be included as part of this invention, provided they come within the scope of the appended claims.

## What is claimed is:

1. A process for treating an aluminum-copper or an aluminum-silicon alloy to improve adhesion of metal layers to said alloy comprising:
  - (a) contacting said alloy with an acidic tin immersion composition to produce a tin immersion coating on said alloy;
  - (b) contacting said tin immersion coating with an etchant to substantially remove said tin immersion coating to produce an etched alloy surface having a microporous structure;
  - (c) further coating said microporous structure with a metal by an immersion metal coating process to yield an immersion metal coated aluminum substrate; and
  - (d) electrolytically coating said immersion metal coated aluminum substrate with a metal.

2. The process of claim 1 for producing a microporous structure on said aluminum alloy wherein said acidic tin immersion composition is a tin immersion composition of matter comprising a compound a divalent tin ion-containing compound, a fluoride ion-containing compound, and an acid hydrogen ion-containing compound.

3. The process of claim 2 further comprising coating said etched alloy with a metal by a zinc immersion metal coating process to obtain a zinc coated aluminum substrate.

4. The process of claim 3 comprising electrolytically coating said zinc coated aluminum substrate with nickel.

5. A product produced by the process of claim 4.

6. The process of claim 5 where said divalent tin ion-containing compound comprises a tin salt, said fluoride ion-containing compound comprises hydrofluoric acid or a fluoride salt, and said acid hydrogen ion-containing compound comprises a mineral acid.

7. The process of claim 6 wherein said divalent tin ion is present in an amount from about 0.05 to about 0.15 mols, said fluoride ion is present in an amount from about 0.25 to about 0.75 mols, and said acid hydrogen ion is present in an amount from about 0.25 to about 0.75 mols.

8. A product produced by the process of claim 7.

9. A product produced by the process of claim 6.

10. A product produced by the process of claim 5.

11. The process of claim 1 comprising further coating said etched alloy with a metal by a zinc immersion metal coating process to yield a zinc coated aluminum substrate.

12. The process of claim 4 comprising electrolytically coating said zinc coated aluminum substrate with nickel.

13. A product made by the process of claim 12.

14. The process of claim 11 comprising electrolytically coating said zinc coated aluminum substrate with nickel.

15. A product produced by the process of claim 4.

16. The process of claim 4 where said aluminum alloy comprises an aluminum-silicon alloy and said etchant comprises a fluoride ion containing etchant.

17. A product made by the process of claim 16.

18. The process of claim 4 where said aluminum alloy comprises an aluminum-copper alloy and said etchant comprises a fluoride ion containing etchant.

19. The process of claim 18 comprising electrolytically coating said zinc coated aluminum substrate with nickel.

20. A product made by the process of claim 19.

21. A product made by the process of claim 18.

\* \* \* \* \*

UNITED STATES PATENT AND TRADEMARK OFFICE  
**CERTIFICATE OF CORRECTION**

PATENT NO. : 5,601,695  
DATED : February 11, 1997  
INVENTOR(S) : MURANUSHI et al.

It is certified that error appears in the above-identified patent and that said Letters Patent is hereby corrected as shown below:

- Claim 2, col. 10, line 4, delete "a compound".  
Claim 5, col. 10, line 1, "claim 4" should read --claim 1--.  
Claim 6, col. 10, line 1, "claim 5" should read --claim 2--.  
Claim 14, col. 10, line 1, "claim 11" should read --claim 1--.  
Claim 18, col. 10, line 1, "claim 4" should read --claim 1--.  
Claim 20, col. 10, line 1, "claim 19" should read --claim 18--.  
Claim 21, col. 18, line 1, "claim 18" should read --claim 19--.

Signed and Sealed this  
Eighth Day of July, 1997



Attest:

BRUCE LEHMAN

Attesting Officer

Commissioner of Patents and Trademarks

UNITED STATES PATENT AND TRADEMARK OFFICE  
**CERTIFICATE OF CORRECTION**

PATENT NO. : 5,601,695  
DATED : February 11, 1997  
INVENTOR(S) : MURANUSHI

Page 1 of 3

It is certified that error appears in the above-identified patent and that said Letters Patent is hereby corrected as shown below:

Claim 2, col. 10, line 4, delete "a compound".

Claim 3, col. 10, line 1, change "3. The process of claim 2" to --5. The process of claim 1--.

Claim 4, col. 10, line 1, change "4. The process of claim 3" to --7. The process of claim 5--.

Claim 5, col. 10, line 1, change "5. A product produced by the process of claim 4" to --9. A product made by the process of claim 1--.

Claim 6, col. 10, line 1, change "6. The process of claim 5" to --3. The process of claim 2--.

Claim 7, col. 10, line 1, change "7. The process of claim 6" to --4. The process of claim 3--.

Claim 8, col. 10, line 1, change "8. A product produced by the process of claim 7" to --10. A product made by the process of claim 2--.

Claim 9, col. 10, line 1, change "9. A product produced by the process of claim 6" to --11. A product made by the process of claim 3--.

Claim 10, col. 10, line 1, change "10. A product produced by the process of claim 5" to --12. A product made by the process of claim 4--.

UNITED STATES PATENT AND TRADEMARK OFFICE  
**CERTIFICATE OF CORRECTION**

PATENT NO. : 5,601,695  
DATED : February 11, 1997  
INVENTOR(S) : MURANUSHI

Page 2 of 3

It is certified that error appears in the above-identified patent and that said Letters Patent is hereby corrected as shown below:

Claim 11, col. 10, line 1, change "11. The process of claim 1" to --6. The process of claim 2--.

Claim 12, col. 10, line 1, change "12. The process of claim 4" to --8. The process of claim 6--.

Claim 13, col. 10, line 1, change "13. A product made by the process of claim 12" to --20. The process of claim 18--.

Claim 14, col. 10, line 1, change "14. The process of claim 11" to --19. The process of claim 18--.

Claim 15, col. 10, line 1, change "15. A product produced by the process of claim 4" to --13. A product made by the process of claim 8--.

Claim 16, col. 10, line 1, change "16. The process of claim 4" to --14. The process of claim 1--.

Claim 17, col. 10, line 1, change "17. A product made by the process of claim 16" to --21. The process of claim 19--.

Claim 18, col. 10, line 1, change "claim 4" to --claim 1--.

Claim 19, col. 10, line 1, change "19. The process of claim 18 comprising elctetrolytically" to --15. The process of claim 5 comprising electrolytically--.

UNITED STATES PATENT AND TRADEMARK OFFICE  
**CERTIFICATE OF CORRECTION**

PATENT NO. : 5,601,695  
DATED : February 11, 1997  
INVENTOR(S) : MURANUSHI

Page 3 of 3

It is certified that error appears in the above-identified patent and that said Letters Patent is hereby corrected as shown below:

Claim 20, col. 10, line 1, change "20. A product made by the process of claim 19" to --16. A product made by the process of claim 14--.

Claim 21, col. 10, line 1, change "21. A product made by the process of claim 18" to --17. A product made by the process of claim 15--.

Signed and Sealed this

Fourteenth Day of October, 1997

Attest:



BRUCE LEHMAN

Attesting Officer

Commissioner of Patents and Trademarks